

# United States Patent Office

2,697,660

Patented Dec. 21, 1954

1

2,697,660

## PURIFICATION OF TITANIUM BY WASHING AND FROTH FLOTATION

Merle E. Sibert, Garfield Heights, Ohio, assignor, by mesne assignments, to the United States of America as represented by the Secretary of the Navy

No Drawing. Application April 25, 1951,  
Serial No. 222,937

1 Claim. (Cl. 75—121)

If titanium contains even very small amounts of foreign materials from the primary stages of reduction to metal, it lacks ductility and necessary workability. Inclusion of such materials can be avoided by a suitable procedure and precautions. For instance, by the process in the application of M. A. Steinberg, M. E. Sibert and A. A. Topinka, Serial No. 202,806, it is possible to produce titanium electrolytically to desired standard of purity. However, where foreign materials have not been avoided it is still possible by the features of the present invention to prepare the metal to proper standards. Thus, titanium carrying materials such as oxide, carbide, and salts by its initial formation can be brought to finished condition providing properly ductile metal. Other objects and advantages of the invention will appear from the following description.

To the accomplishment of the foregoing and related ends, said invention then comprises the features hereinafter fully described and particularly pointed out in the claim, the following description setting forth in detail certain illustrative embodiments of the invention, these being indicative, however, of but a few of the various ways in which the principle of the invention may be employed.

In such electrolytic preparation of titanium in an alkaline earth chloride fused bath, for example, the titanium deposits on the cathode in the form of a black spongy mass, admixed with impurities such as alkaline earth halide from the electrolytic bath, other calcium compounds, including calcium carbide, carbon if graphite be present in the cell, titanium carbide, and titanium monoxide. Carbon in combined or free form, and oxides, are especially detrimental, as titanium metal is peculiar in that very small amounts of carbon and oxygen render the metal so hard and brittle that it cannot be mechanically worked. In the present process, the titanium metal is prepared in a manner to be freed from such detrimental materials and be formed as a finished product which is ductile. If titanium metal powder be fused in the presence of carbon or oxygen or both, these latter elements go into solid solution in titanium and no method is known for mechanical separation after such fusion has taken place. X-ray diffraction examination shows that in electrolytically formed titanium according to the present invention, carbon and oxygen, if present, are separate entities, and these can be removed mechanically in operations leading up to the ultimate fusion and formation of ductile metal.

In a typical case, the titanium develops in the primary stage of reduction as a loose black spongy mass. This I give a primary wash in warm water at a temperature of about 60° C. to remove most of the free calcium chloride. When wetted, some areas of the deposit appear black and others grey. These black areas are heavy in titanium carbide and generally the extreme upper and lower tenths of the material exhibit this character. These carbided areas preferably are sliced or sawed off and treated separately from the major relative pure portions.

The material is next dispersed in about 20 times its volume of pure water and heated to the boiling point for 30 to 60 minutes with vigorous agitation. Free carbon floats to the surface and may be skimmed off. This vigorous washing step removes occluded salts, such as chloride, from the deposit, and also converts any calcium metal or calcium carbide which may be present to calcium hydroxide. An acid not attacking the titanium but solubilizing the calcium hydroxide is then added to

2

the wash water to a pH of 4.5 to 5.0. Such acid thus is not a strong mineral acid, but a weak organic acid, as formic, acetic, citric, and the like. The metal particles are then allowed to settle to the bottom of the container and the supernatant liquid is decanted off. This supernatant liquid carries finely divided titanium carbide in suspension and the most of this extremely fine titanium carbide may be removed by decanting two or three times. The residual titanium metal is then filtered and ground wet to 60 to 80 mesh in order to free any occluded impurities, and the washing cycle described above including formic acid treatment is repeated. This final treatment removes all traces of calcium chloride, calcium hydroxide, calcium oxide, calcium metal, and calcium carbide. In general, such a procedure is effective in providing commercially pure titanium metal suitable for direct melting, where the initial electrolytic processing has been carried out properly. However, if electrolytic processing is such that any undue amount of titanium carbide or titanium monoxide remains with the deposited metal, then it is necessary to examine the material analytically to determine the extent of the carbide and oxide contents. If titanium monoxide is present at all, that is in amounts greater than a few hundredths of a percent or if carbide is present to the extent of 1% or more, then further separation is necessary.

In order to accomplish this separation, the powdered metal is ground in a stainless steel ball mill in water to approximately —325 mesh and the slurry which is obtained is again treated with water and formic acid washes as before to provide insurance of as complete a calcium and carbon removal as possible. The residue which is obtained is filtered and is then dried in a vacuum. Then any residual titanium monoxide or titanium carbide may be separated by a further step.

A usual type froth flotation cell (for example the Fagergren cell) is suitable. The oxide and carbide separation steps are handled consecutively. In the case of oxide or carbide, the concentration of starting power may be between 10 and 20% by weight of the total solution. With traces of calcium salts present, if it be attempted to apply flotation procedures to such a system, all of the ingredients float out of the cell without any separation. Fundamentally, it appears that this is due to the occlusion of the particles without regard to composition, such occlusion being made effective by the multivalent ion  $\text{Ca}^{2+}$ . I have found that agents capable of insolubilizing or de-ionizing or sequestering calcium obviate this, and by thus conditioning the material, make possible the desired separation, the detrimental components being floated off, while the titanium metal remains, being in effect depressed. Especially desirable are water-soluble phosphates and glasses of the pyro-metaphosphate system. Also sulphonated fatty alcohols, their esters, and their derivatives. Frothing agents from the class of higher alcohols may also be used. The alkali metal salts of the xanthic acids are most useful as collecting agents. The crude titanium powder is dispersed in a 0.5 to 1% solution of, for example, tetrasodium pyrophosphate, and a collecting agent such as potassium ethyl xanthate in ethyl chlor-carbonate is added to the extent of 2½ milliliters per liter of solution. The mixture is then conditioned in the cell for 10 to 15 minutes and flotation is initiated. Titanium monoxide concentrates in the froth. Usually 2 to 3 passes are sufficient to remove all titanium monoxide present to the extent that it may be encountered in electrolytic titanium. (It should again be pointed out that if the conditions of the electrolysis are sufficiently good the titanium monoxide step such as just described is not necessary.)

If any amount of carbide in the form of titanium carbide is present in the deposit of titanium metal, this is removed by a flotation step. For this separation, again the concentration of crude titanium metal powder may be of the order of 10 to 20 parts by weight in the frothing solution and the solution consists primarily of a 12 to 15% solution of a complex water soluble phosphate sequestering agent, e. g., tetrasodium pyrophosphate dehydrate. Again in this case, the titanium metal is depressed and the titanium carbide floats.

After conditioning for several minutes, the carbide is

allowed to float off. It is important to note that separate frothers are not required since in this concentration, tetrasodium pyrophosphate is in itself a sufficient frother in view of its detergent properties. Under normal conditions, the titanium carbide may be separated completely in 3 to 4 passes, but the process may be facilitated by use of acid media at pH of the order of 2.0 to 2.5. The acid used should be such as does not attack the titanium, as mentioned above. Thus, while hydrofluoric acid is satisfactory to a limited extent in rubber lined tanks, it has the drawback that if the concentration be too high, reaction occurs on the metal and efficiency of recovery is correspondingly reduced. Phosphoric acid is particularly satisfactory, and a clean separation of titanium carbide from titanium metal may be obtained in the presence of this agent in one to two passes. Both in the case of the titanium monoxide and titanium carbide separation, the titanium metal is recovered by washing and filtration, followed by vacuum drying.

Electrolytically formed titanium metal subjected to this washing and flotation procedure shows a titanium metal content of 99.95% titanium, or better.

In order to produce metal of a commercially useful nature from such powder, the dry powder is pressed into pellets and fused in a vacuum or in an inert atmosphere arc furnace. Such metal is malleable and forgeable, because of its high purity and low oxygen content, and it may be worked by all usual methods applicable to ductile metals.

The following examples are illustrative:

I. 125 grams of titanium metal powder containing 20% titanium monoxide by weight was ground in water to a -325 mesh powder in a stainless steel ball mill. The dispersion was diluted to a volume of 1 liter with distilled water, and 3½ grams of tetrasodium pyrophosphate was added, and 2½ cc. of potassium ethyl xanthate in a suitable organic solvent (such as ethyl chlor-carbonate). This was maintained at room temperature and treated in a froth flotation chamber of the Fahrenren type. Conditioning was accomplished by running the chamber at low speeds or under conditions where air intake was shut off for a period of about 10 minutes. The air intake valve was then opened and flotation carried out for a period of about 15 minutes. Both the residue and the froth were again treated separately, resulting in a concentrate, a middles, and a froth tails. The middles were again treated resulting in a depressed concentrate, a middles, and a froth tails. The depressed concentrate was added to the various concentrates obtained in the foregoing description and the froths also collected and combined. After washing and drying, 90 grams of metallic concentrate were obtained and 35 grams of froth concentrate. Analysis indicated that the titanium concentrate was substantially chemically pure, indicating a flotation efficiency of the order of 90%, whereas the material obtained in the froth fraction contains approximately 70% titanium monoxide and 30% titanium metal.

The metal concentrate thus obtained after drying, compressing, and melting was malleable and ductile.

II. 125 grams of titanium metal containing 20% by weight of titanium carbide was ground in water in a stainless steel ball mill to -325 mesh. The slurry was removed and diluted to 1 liter with distilled water. 50 grams of tetrasodium pyrophosphate was added and the slurry thus obtained was treated in a Fahrenren cell. After conditioning for 10 minutes in the manner as described in Example I, the material was then vigorously floated for 15 minutes, resulting in a metal concentrate which remained in the cell and a froth high in titanium carbide. The metal concentrate was retreated twice more and all of the froths were collected. Finally the froth

was given a double treatment with the addition of 20 more grams of tetrasodium pyrophosphate. After combining the metal concentrates and the various froth tails, a yield of 92 grams of metal was obtained, which on compressing, fusion, and rolling was ductile, indicating the substantial absence of titanium carbide. The titanium carbide content of the froth was of the order of 76%, thus showing a metal recovering at least of the order of 90%. (The pH during frothing was 10.5.)

10 III. Using starting agents having higher or lower percentages of tetrasodium pyrophosphate in the first roughing such as 60 grams of tetrasodium pyrophosphate per liter or 40 grams of tetrasodium pyrophosphate per liter gave results such that the yield of metal was between 80 15 and 85% in a high state of purity. In these particular cases, the frothing time was considerably longer, and at least one more cycle was required to obtain such a state of purity. The initial roughing concentrate makeup of 50 grams of tetrasodium pyrophosphate per liter is somewhat critical for best results. The pH during frothing was 10.5.

20 IV. 125 grams of titanium metal containing 20% of titanium carbide was prepared as indicated in the foregoing, and 48 grams of tetrasodium pyrophosphate were 25 added. Sufficient phosphoric acid was then added to the batch so that a pH of 2.0 was reached. The material was then conditioned for about 10 minutes. The flotation time was about 15 minutes. A countercurrent cycle involving at most two passes was sufficient to develop a 30 yield of 85 to 90% metal of satisfactory commercial purity.

35 Other modes of applying the principle of the invention may be employed, change being made as regards the details described, provided the features stated in the following claim or the equivalent of such be employed.

I therefore particularly point out and distinctly claim as my invention:

40 The method of recovering titanium metal from a cathode deposit obtained by electrolytic decomposition of titanium monoxide in a fused halide salt bath which comprises removing halide salt adhering to the titanium metal deposit by washing first with water and then with an acidic aqueous medium, and thereafter removing any 45 titanium monoxide and titanium carbide admixed with the titanium metal deposit by grinding the washed deposit and by subjecting the ground deposit to froth flotation separation in the presence of a water soluble phosphate, and a collecting agent for titanium oxide, and recovering the residual metallic titanium.

#### References Cited in the file of this patent

#### UNITED STATES PATENTS

| Number       | Name              | Date          |
|--------------|-------------------|---------------|
| 55 2,205,854 | Kroll             | June 25, 1940 |
| 2,274,237    | Jaeger et al.     | Feb. 24, 1942 |
| 2,537,068    | Lillendahl        | Jan. 9, 1951  |
| 2,543,399    | Calingaert et al. | Feb. 27, 1951 |
| 2,543,407    | Hill et al.       | Feb. 27, 1951 |
| 60 2,553,444 | Dunn et al.       | May 15, 1951  |
| 2,557,455    | Moyer             | June 19, 1951 |

#### FOREIGN PATENTS

| Number   | Country       | Date    |
|----------|---------------|---------|
| 65 8,567 | Great Britain | of 1907 |
| 13,759   | Great Britain | of 1904 |

#### OTHER REFERENCES

70 Taggart, Handbook of Mineral Dressing (c) 1945, sec. 12, page 34. (Copy in Div. 55.)